

Patented Feb. 4, 1947

2,415,169

# UNITED STATES PATENT OFFICE

2,415,169

## ELECTRODEPOSITION OF LEAD

Allen G. Gray, Rocky River, Ohio, assignor to  
E. I. du Pont de Nemours & Company, Wil-  
mington, Del., a corporation of Delaware

No Drawing. Application September 22, 1942,  
Serial No. 459,282

11 Claims. (Cl. 204—53)

1

This invention relates to electrodeposition and more particularly to improved compositions and processes for electrodepositing lead. Ideally, the invention consists in dry, free-flowing lead sulfamate plating compositions which preferably contain an anthraquinone sulfonate, and in lead plating processes wherein such compositions are employed.

Systems for electrodepositing lead have heretofore been restricted in their usefulness through their lack of ability to produce a good initial deposit in low current density areas upon the cathode. This inability, commonly referred to as lack of "covering power," is especially pronounced when the cathode is such a metal as cast iron or malleable iron or certain alloy steels. Failure to secure adequate coverage is a particularly serious objection when the cathode is being lead plated to protect it against corrosion.

It is an object of the present invention to provide improved compositions and processes for the electrodeposition of lead over a wide range of current densities and particularly having good covering power at low current densities. A further object is to provide compositions and processes for the production of dense, adherent, non-porous, and ductile electrodeposits of lead. A further object is to provide lead plating compositions which are dry, free-flowing, and readily soluble in water, and which are particularly adapted to the preparation of novel plating baths having improved covering power in low current density ranges. Further objects will appear hereinafter.

The foregoing and other objects of this invention are accomplished by processes in which lead is electrodeposited in the presence of an anthraquinone sulfonate, and are further accomplished by dry electrodepositing compositions and by electrodepositing solutions in which an anthraquinone sulfonate is present. The objects are accomplished with especial success by lead sulfamate electroplating solutions in which an anthraquinone sulfonate is present, and by dry solid products comprising dry reaction mixtures of litharge and sulfamic acid suitable for dissolution in water to give such electroplating baths.

The processes and compositions of this invention are characterized by their ability to effect deposition of lead at low current densities. The benefits of the invention are obtained with lead plating baths over a wide pH range, but are especially apparent in acid plating systems, that is, in electroplating compositions and baths having a pH lower than about 7, and especially below about 4.2. In such acid systems the difficulty of getting adequate coverage at low current densities is more pronounced than in alkaline baths and the benefits to be derived from the inclusion of an anthraquinone sulfonate are enhanced.

5

10

15

20

25

30

35

40

45

50

55

60

2

According to this invention any anthraquinone sulfonate may be employed in an electrodepositing composition. There may be used, for instance, monosulfonic acids such as 1-anthraquinone sulfonic acid or 2-anthraquinone sulfonic acid or polysulfonic acids such as 1,8-anthraquinone disulfonic acid or 2,7-anthraquinone disulfonic acid. The bath-soluble salts of the sulfonic acids such as the sodium, potassium, or ammonium salts or partial salts, may suitably be used, and because of their excellent solubility, ease of preparation, and ease of handling in dry form, the sodium salts of the sulfonic acids may be preferred. The manner of adding the sulfonic acid is comparatively unimportant since whether the addition agent is present as an acid or as a salt or as a partial salt will depend upon the pH of the bath. For purposes of this description where reference is made to a sulfonate, it will be understood that this may be a salt or partial salt or the free acid.

The amount of an anthraquinone sulfonate to include in an electroplating composition or bath will vary depending upon the plating system involved, the metal being plated, the magnitude of effect desired, and other similar factors. The amount can best be determined by a few simple tests in the particular bath to be used. In general it will be found that from about .05 to 5.0 grams per liter of anthraquinone sulfonate will be satisfactory.

Anthraquinone sulfonates may be used in electroplating baths in combination with other addition agents. By far the best results are obtained by the use of a sulfite cellulose waste which co-acts with the anthraquinone sulfonate to produce excellent results. Sulfite cellulose waste is a well known commodity of commerce and it has previously been found useful in certain plating systems as an addition agent in its own right. Lignin sulfonic acid, derived from sulfite cellulose waste, may be used instead with substantially equivalent results. This and other derivatives of a similar nature are known to be equivalent to sulfite cellulose waste and they require no extended discussion.

When a second addition agent is used in combination with the anthraquinone sulfonate the amount of the second addition may also be considerably varied. For instance, when the second agent is sulfite cellulose waste, the amount used may vary from about .25 to 15 grams per liter and more preferably from about 1 to 5 grams per liter.

When reference is made herein to electrodeposition of lead it will be understood that the lead may be co-deposited with another metal or metals to produce alloys. The invention is applicable, for instance, in the co-electrodeposition of lead and antimony.

Benefits are obtained by using an anthraquinone sulfonate in any lead electrodepositing bath according to the present invention. As already noted above the improvement is particularly apparent in acid plating systems, but neutral or alkaline baths may also be modified to advantage. Typical of lead-plating baths which may be modified by the inclusion of an anthraquinone sulfonate are the fluoborate, sulfamate, and fluosilicate baths described in the following examples. Other baths which may be modified are, for instance, the acetate bath (Metal Finishing 38, 533 (1940)) containing 10 gm.



12 to 16 gm.  $\text{Na}(\text{C}_2\text{H}_3\text{O}_2)_2 \cdot 3\text{H}_2\text{O}$ , 2 gm. acetic acid, .4 to .6 gm. glue, and 3 to 4 drops cresol per 100 ml. solution; the perchlorate bath (Trans. Am. Electrochem. Soc. 23, 159 (1913)) containing 5% lead, 2 to 5% free perchloric acid, and .05% peptone; and baths having as a principal electrolyte lead nitrate, lead oxalate, lead dithionite, lead cyanide, or sodium plumbite.

The invention will be better understood by reference to the following illustrative examples:

*Example I*

A lead fluoborate electroplating bath was prepared as described in the Transactions of the Electrochemical Society, vol. 36, page 243, having the following composition:

|                                  | Grams/liter |
|----------------------------------|-------------|
| Hydrofluoric acid (50% solution) | 160         |
| Boric acid                       | 74.4        |
| Basic lead carbonate             | 129         |
| Glue                             | 0.1         |

To this aqueous solution there was added 0.2 gram/liter of 1-anthraquinone sodium sulfonate to obtain a bath of this invention.

Copper test plates were electroplated in this solution at various current densities. It was found that complete coverage of the test plate with lead was effected in one minute at all current densities including current densities as low as 0.1 amp./sq. ft. On the other hand similar test plates electroplated in the solution before the addition of the 1-anthraquinone sodium sulfonate were not covered in one minute at current densities below 7.0 amp./sq. ft. It will be seen therefore that the inclusion of the anthraquinone sulfonate effected a remarkable improvement in the coverage at low current density.

*Example II*

A lead plating solution was made up having the following composition:

|                                  | Grams/liter |
|----------------------------------|-------------|
| Litharge                         | 150         |
| Sulfamic acid                    | 150         |
| Ammonium sulfamate               | 75          |
| 1-anthraquinone sodium sulfonate | 0.5         |
| Sulfite cellulose waste          | 5           |

The solution had a pH of 1.5.

Copper test plates were lead plated in this solution at various current densities. A smooth, dense, lustrous deposit was secured in one minute at current densities as low as 0.9 amp./sq. ft. Test plates which were electroplated with lead in a solution having similar compositions, except that the 1-anthraquinone sodium sulfonate was omitted, gave no coverage in one minute at current densities below 5 amp./sq. ft.

*Example III*

A bath was made up having the same compo-

sition as in Example II above, except that instead of 1-anthraquinone sodium sulfonate, there was used as the addition agent 1,8-anthraquinone sodium disulfonate. The test plates showed that without the anthraquinone disulfonate, coverage was incomplete in one minute at current densities below 5 amp./sq. ft., whereas with the anthraquinone disulfonate, coverage was complete at current densities as low as 2 amp./sq. ft.

It will be seen from the above examples that a substantial improvement in covering power of certain lead electroplating baths is effected by the inclusion therein of an anthraquinone sulfonate. This improvement is noted also in other lead electroplating baths, such as the fluosilicate or acetate baths. A typical lead fluosilicate bath in which improvement is effected is shown in "Plating and Finishing Guidebook" (1941) p. 48, bath No. II, having the composition:

|                       | Grams/liter |
|-----------------------|-------------|
| Lead fluosilicate     | 150         |
| Free fluosilicic acid | 30          |
| Glue                  | 3           |

The benefits of this invention are particularly noticed in lead sulfamate electroplating baths. Plating compositions especially suited for making up such baths are the reaction products obtained by mixed lead compounds with sulfamic acid in the absence of substantial amounts of water. Such compositions may be produced, for instance, by mixing litharge, solid dry sulfamic acid, and ammonium sulfamate in the presence of traces (for instance 0.5 to 2.0 per cent by weight) of water and at a temperature of about from 105-145° F., whereby a reaction occurs between litharge, acid, and ammonium sulfamate as is evidenced by a change in color of the mixture from that of the litharge to substantially white. A plating composition of superior properties is obtained as a dry, very readily water soluble, free-flowing product.

The proportions of litharge and sulfamic acid used in making the dry reaction product should be about those required to give a bath of the desired characteristics when the product is dissolved in water at a concentration such as indicated in Example II above. Thus, the proportions should be such as to give a pH of less than 7 and preferably, less than 4.2. The amount of ammonium sulfamate should be appreciable, but not the major proportion of the product, comprising about from 5 to 30% of the mixture. A preferred mixture might contain, for instance, the reacted equivalent of about 40 parts of litharge, 40 parts of sulfamic acid and 20 parts of ammonium sulfamate, but it will be understood that these proportions are susceptible to considerable variation.

By including an anthraquinone sulfonate and, optionally, another addition agent such as sulfite cellulose waste, in a dry lead sulfamate or litharge-sulfamic acid reaction product, there is obtained a complete, balanced product which is ideally suited for use by the trade. Such a product, for instance, may readily be dissolved in water to give lead plating solutions of this invention without the inconvenience of measuring out or weighing the separate constituents.

By dissolving a suitable sulfamate-lead composition, such as for instance one of the above-described compositions in a proper amount of water, there may be produced a lead sulfamate plating bath which is particularly amenable to the action of an anthraquinone sulfonate in ac-

cordance with this invention. Such a solution will generally contain from about 50 to 400 grams/liter of dissolved lead (expressed as Pb) and preferably from about 100 to 200 grams/liter. The total sulfamate content will usually be equivalent to from about 50 to 450 grams/liter of sulfamic acid and preferably from about 100 to 250 grams/liter.

The weight ratio of combined lead content, expressed as Pb, to lead sulfamate plus free sulfamic acid content is important. The weight ratio of combined Pb to  $(\text{NH}_2\text{SO}_3\text{Pb} + \text{NH}_2\text{SO}_3\text{H})$  should be from about 1:1 to 1:3 and preferably about 1:2. The amount of free sulfamic acid present in the bath should be from about 10 to 40 grams/liter. It will be understood that there will preferably be present sulfamate in combination as ammonium sulfamate and that this sulfamate is in addition to the lead sulfamate and sulfamic acid. The ammonium sulfamate content preferably will be from about 25 to 100 grams/liter.

Lead sulfamate plating baths in which anthraquinone sulfonates are particularly effective are definitely acidic. The pH should ordinarily be from about 0.1 to about 4.2 and preferably should be from 1.0 to 3.0. Particularly excellent results have been obtained using a pH of about 1.3 to 2.0. If in making up the bath sulfamic acid is used as such, the pH may be adjusted by appropriate additions of sulfamic acid. If part or all of the sulfamic acid is added to the bath in the form of a salt, then the pH may be adjusted by the use of another acid such as formic acid, acetic acid, or nitric acid.

In the operation of the lead sulfamate bath lead anodes are used to replenish the lead content of the solution and maintain the composition as above indicated, but in some instances it may be found convenient to adjust the composition of the bath by appropriate additions of basic lead compositions such as litharge and by the addition of sulfamic acid.

While certain illustrative compositions and processes have been shown, it will be understood that the invention is not limited thereby but that one skilled in the art, without departing from the spirit of the invention, may readily devise numerous compositions and processes for the electrodeposition of lead.

I claim:

1. In a process for the electrodeposition of lead, the step comprising effecting electrodeposition of lead from an acidic, aqueous lead electrodepositing solution in the presence of about from .05 to 5.0 grams per liter of an anthraquinone sulfonate and 1.0 to 5.0 grams per liter of sulfite cellulose waste.

2. In a process for the electrodeposition of lead, the step comprising effecting electrodeposition of lead from an aqueous solution containing about from 50 to 400 grams per liter of lead, 50 to 450 grams per liter of sulfamic acid, .05 to 5.0 grams per liter of an anthraquinone sulfonate, and from 1.0 to 5.0 grams per liter of sulfite cellulose waste.

3. A lead electrodepositing composition in dry form, comprising a lead compound and an anthraquinone sulfonate, the proportions of anthraquinone sulfonate and other constituents being such that when the composition is dissolved in water to make a solution of suitable concentration for electroplating, the anthraquinone is present in the solution at a concentration of from .05 to 5.0 grams per liter.

4. A lead electrodepositing composition in dry form, comprising a lead sulfamate and an anthraquinone sulfonate, the proportions of anthraquinone sulfonate and other constituents being such that when the composition is dissolved in water to make a solution of suitable concentration for electroplating, the anthraquinone is present in the solution at a concentration of from .05 to 5.0 grams per liter.

5. A lead electrodepositing composition in dry form comprising litharge, sulfamic acid, and an anthraquinone sulfonate, the proportions of anthraquinone sulfonate and other constituents being such that when the composition is dissolved in water to make a solution of suitable concentration for electroplating, the anthraquinone is present in the solution at a concentration of from .05 to 5.0 grams per liter.

6. A lead electrodepositing composition in dry form comprising litharge, sulfamic acid, an anthraquinone sulfonate, and sulfite cellulose waste, the proportions of anthraquinone sulfonate and other constituents being such that when the composition is dissolved in water to make a solution of suitable concentration for electroplating, the anthraquinone is present in the solution at a concentration of from .05 to 5.0 grams per liter.

7. An aqueous lead sulfamate plating solution comprising an anthraquinone sulfonate, in a concentration of about from 0.5 to 5.0 grams per liter ammonium sulfamate, and the reaction product of such proportions of litharge and sulfamic acid as to give a pH of from about 0.1 to 4.2 in the bath.

8. An aqueous lead sulfamate plating solution comprising 1-anthraquinone sodium sulfonate in a concentration of about from .05 to 5.0 grams per liter and the reaction product of about 40 parts by weight of litharge, 40 parts of sulfamic acid, and 20 parts of ammonium sulfamate.

9. In a process for the electrodeposition of lead, the step comprising effecting electrodeposition of lead from an aqueous lead electrodepositing solution in the presence of about from 0.05 to 5.0 grams per liter of an anthraquinone sulfonate.

10. In a process for the electrodeposition of lead, the step comprising effecting electrodeposition of lead from an aqueous lead sulfamate electrodepositing solution in the presence of about from 0.05 to 5.0 grams per liter of an anthraquinone sulfonate.

11. In a process for the electrodeposition of lead, the step comprising effecting electrodeposition of lead from an aqueous lead fluoroborate electrodepositing solution in the presence of about from 0.05 to 5.0 grams per liter of an anthraquinone sulfonate.

ALLEN G. GRAY.

#### REFERENCES CITED

The following references are of record in the file of this patent:

#### UNITED STATES PATENTS

| Number    | Name          | Date          |
|-----------|---------------|---------------|
| 2,271,209 | Schlotter     | Jan. 27, 1942 |
| 2,294,053 | Stack, et al. | Aug. 25, 1942 |
| 1,515,042 | Heck          | Nov. 11, 1924 |
| 2,318,592 | Cupery        | May 11, 1943  |

#### OTHER REFERENCES

Trans. Electrochem. Society, vol. 76 (1939)  
page 371, copy in Div. 56.